

Aug. 2, 1927.

1,637,793

M. C. VANDER KAMP

METHOD OF FINISHING METAL WALLS

Filed May 21, 1925



Inventor.  
M. C. Vander Kamp.  
By Dewey Strong  
Towle and Loftus  
Attorneys.

## UNITED STATES PATENT OFFICE.

MARTIN C. VAN DER KAMP, OF SAN JOSE, CALIFORNIA.

## METHOD OF FINISHING METAL WALLS.

Application filed May 21, 1925. Serial No. 31,858.

This invention relates particularly to a method of holding tile and like compositions onto a surface of metal and the invention relates especially to such a method, whereby the metal walls of the rooms of a ship can be formed and decorated in much the same manner as walls formed from other material are now decorated in hotels and like structures. Plaster and like compositions will not adhere to metal surfaces such as the metal walls of rooms on ships and therefore where such walls are covered at all, it is necessary to drill into or through the walls to secure a holding support thereto. Wood panel work is the usual material used in covering such walls. This panel work is not only very expensive to install, but also forms a great fire hazard. It is the primary object of my invention to provide a method whereby these metal walls can be easily covered with the desired covering and decorating material in a manner similar to that now used on other walls.

With the above and other objects in view, my invention consists in the features of construction and operation set forth in the following specification and illustrated in the accompanying drawing. In such drawing annexed hereto and forming a part of this specification, I have shown one specific embodiment of my invention but it will be understood that the invention can be otherwise embodied and that the drawing is not to be construed as defining or limiting the scope of the invention, the claims appended to this specification being relied upon for that purpose.

The figure in the drawing illustrates one specific embodiment of my invention.

The floors of bathrooms and often the walls thereof, are finished with blocks or tiles laid in cement. The walls of other rooms are usually covered with a coating of plaster or mortar, which coating is thereafter papered or decorated as desired. This outer layer is mounted on a thicker layer of a coarse plastic material secured to the floor or wall. As stated above, such material will not adhere to a metal surface and therefore the metal walls of ships have not been thus finished and decorated. My invention aims to provide a method for overcoming this objection, thereby greatly improving the interior decoration of ships and at less expense than the cost of the present decorating thereof.

I have contemplated the covering of these metal walls with a material such as will support the outer finishing layer, mortar, tiles, or the like. The difficulty however has been to secure such material to the metal. After considerable experimenting I have found that asphalt adheres with great security to metal and also to material formed from plastic compositions. Upon further experiment I have found that by forming the desired wall covering material into flat blocks of a uniform thickness and providing a coating of heated asphalt to one of the cooperating surfaces of the blocks and metal, the blocks will adhere to the metal with great security. A metal wall can thereby be entirely covered with a material to which the usual finishing layer of mortar, tiles etc. can be applied in the usual manner.

Various plastic materials and tiles formed therefrom are today being used as veneers or coatings for walls, floors, etc. in building construction. I have herein specially contemplated the use of magnesite plastic material for this purpose, and particularly the application of such material to metal floors and walls, because of its elasticity and its quality of adhering so securely to asphalt, the quality of elasticity being particularly desirable on ship walls because of the warping and weaving movement of such walls I have found that this material like other material of a similar nature will not make a permanent bond with the metal surface. As stated above, however, I have found that by applying a layer of heated asphalt between the surfaces, prior to uniting the same, the two materials are securely and permanently bonded together whatever may be the character of their surfaces. The accompanying drawing illustrates the use of this invention in connection with two such surfaces.

In the drawings, the metal plate 1 may be a wall, a floor, or any other like surface. A layer 2 of covering material is secured to the plate 1 by an intermediate coating of heated asphalt 4. As above stated, this layer 2 comprises a plurality of flat blocks molded from the desired covering material, this material preferably being magnesite for the reasons stated. A finishing layer of mortar, tiles, or any desired material can be provided over the layer 2. In the drawing I have illustrated the finishing layer as being formed of tiling 3, which may be secured

2  
to the outer surface of the layer 2 by a layer 5 of cement, asphalt, or any other suitable adhesive. When the outer finishing layer of mortar or the like is applied in a plastic state, the same adheres to the layer 2 in the usual manner without any intermediate adhesive material.

As will be obvious, my invention provides a method whereby metal walls can be finished off in like manner as have been other walls heretofore. The asphalt furthermore not only provides a firm bond between the metal and layer 2 of covering material, but the asphalt is also plastic and flexible, thereby adapting the same particularly for use on ships and wherever the walls or floors are subjected to movement. Furthermore, the magnesite covering also being flexible, cooperates with the asphalt to form a covering which will adhere to the wall or floor even though the same are subjected to considerable movement.

Having thus described my invention, what

I claim and desire to secure by Letters Patent is:

1. A method of finishing metal walls of ships, comprising forming a coating layer over the wall to be finished of an elastic binding agent, arranging blocks of magnesite material on said binding agent whereby to cement the blocks to the wall, and then forming a finish coating on the exterior surface of said magnesite blocks.

2. A method of finishing metal walls of ships, which comprises forming a comparatively thin layer of an elastic binding agent over the wall to be finished, said binding agent consisting of an asphalt composition in a heated condition, then placing blocks of magnesite material on the wall over said coating to cement the blocks to the wall, forming a coating of a binding agent over said blocks, and then applying a finish to the blocks, the finish adhering to the blocks due to the provision of the binding agent.

MARTIN C. VAN DER KAMP.